

# UNITED STATES PATENT OFFICE.

EDWIN EDSER, HENRY LIVINGSTONE SULMAN, AND FRANK BUTLER JONES, OF LONDON, ENGLAND, ASSIGNORS TO MINERALS SEPARATION NORTH AMERICAN CORPORATION, OF NEW YORK, N. Y.

## TREATMENT OF MATERIALS CONTAINING COAL.

1,418,547.

Specification of Letters Patent. Patented June 6, 1922.

No Drawing.

Application filed November 12, 1920. Serial No. 423,610.

To all whom it may concern:

Be it known that we, EDWIN EDSER, residing at Brockley, London, England, HENRY LIVINGSTONE SULMAN, and FRANK BUTLER JONES, both residing at London, England, all subjects of the King of England, have invented certain new and useful Improvements in the Treatment of Materials Containing Coal, of which the following is a specification.

This invention consists in improvements in or relating to the treatment of materials containing coal, such as poor coal, dross, coal refuse, or washings from coal plant, by a froth-flotation process of concentration, and the present invention relates particularly to the treatment of poor coal containing—

- (a) good coal,
- (b) carboniferous shale or bone coal, and
- (c) gangue or earthy matter, such as clay, carbonates, rocky interlaminations and the like.

Broadly speaking, in the application of the froth-flotation process to the recovery of coal from coal-bearing materials, the powdered material, suspended in liquid, is subjected to agitation and aeration to disseminate minute air bubbles throughout the liquid in such a way that the coal particles are caught in the air-water surface of the bubbles and floated in the form of a froth, and thereby separated from the material which is not caught by the bubbles.

In the froth-flotation process it is well-known that there may be added to the liquid a frothing agent, such as oil.

In the practical application of the froth-flotation process it is also known to add to the liquid a modifying or deflocculating agent which causes the water effectively to wet the gangue particles and prevents these gangue particles from adhering to the gaseous bubbles.

Many agents which are effective as frothing agents are soluble in water or miscible with water. On the other hand, many frothing agents are insoluble or immiscible in water: this is particularly true of oily substances.

We have found that if the frothing agent employed is soluble in water or miscible with water, the tendency is for the froth to

contain only the good coal and not to contain any bone coal or gangue.

55

Certain of the shales, however, such as highly carbonized shales, or bone coal, are useful for their calorific value, and it has been found that by the employment of a certain limited proportion of immiscible oil, such as kerosene oil, in the agent, the highly carbonaceous shale, or bone coal, can also be floated to the exclusion of the gangue.

60

According to the present invention, therefore, a process for the differential separation of the constituents of a coal of the type above referred to consists in subjecting the powdered material, suspended in liquid, to agitation and aeration first in the presence of a soluble frothing agent so as to disseminate minute air bubbles throughout the liquid in such a way that the particles of good coal are floated in the form of a froth, after which a minute quantity of an immiscible or oily agent is added to the pulp, which is again subjected to agitation and aeration to ensure the flotation of the shale or bone coal.

65

Among the soluble frothing agents which can be used to ensure the differential flotation of good coal, cresol (cresylic acid) may be mentioned as an example.

70

The apparatus in which this process is carried out may be any of the known types of apparatus which are at present used in the froth-flotation process of concentrating ores.

75

The following example illustrates the application of this process.

The material used in this test was an Indian bituminous coal which contained 16.1% of ash and gave 12000 British thermal units per lb. In a test on this material 1200 grammes were crushed to pass a screen of 20 meshes to the linear inch and were mixed with water to form a 4:1 pulp. The pulp was placed in a laboratory flotation machine of the sub-aeration type. It was agitated and aerated in the usual way. In order to ensure the production of a first concentrate containing pure coal, a soluble frothing agent was added consisting of cresol at the rate of  $\frac{7}{10}$ ths lb. per ton of crude material. The first froth concentrate amounted to 57.2% of the original and contained only 9.3% of ash, and gave 13075 B. T. U. per lb.

80

85

90

95

100

105

In order now to recover the bone coal or carbonaceous shale there was added to the pulp an agent containing  $\frac{2}{15}$ ths lb. of cresol per ton of crude material and  $\frac{3}{10}$ ths lb. of kerosene oil per ton of crude material. The result was a second froth which contained 35.8% of the original sample, containing 20.8% of ash and giving 11292 B. T. U. per lb. The residue comprising 7% of the original, contained 58% of ash and gave only a trifling calorific value.

In this test the circuit was neutral.

What we claim as our invention and desire to secure by Letters Patent is:—

- 15 1. A process of concentrating impure coal containing good coal, bone coal, and gangue, which consists in subjecting the material to froth-flotation separation with a soluble frothing agent to yield a concentrate relatively high in pure coal and subjecting the remaining pulp to further froth flotation with a frothing agent which includes an insoluble selecting agent to yield a concentrate relatively high in bone coal.
- 20 2. A process of concentrating impure coal containing good coal, bone coal, and

gangue, which consists in subjecting the material to froth-flotation separation with a soluble frothing agent to yield a concentrate relatively high in pure coal and subjecting the remaining pulp to further froth-flotation with a frothing agent which includes an insoluble oil to yield a concentrate relatively high in bone coal.

3. A process of concentrating impure coal containing good coal, bone coal, and gangue, which consists in subjecting the material to froth-flotation separation with cresol to yield a concentrate relatively high in pure coal and subjecting the remaining pulp to further froth-flotation with a frothing agent which includes an insoluble oil to yield a concentrate relatively high in bone coal.

In testimony whereof we have signed our names to this specification in the presence of two subscribing witnesses.

EDWIN EDSER.

HENRY LIVINGSTONE SULMAN.

FRANK BUTLER JONES.

Witnesses:

J. WATT,

LILIAN M. HALLAM.